

## UNITED STATES PATENT OFFICE.

MARTIN WADDELL AND HENRY COWAN WATSON, OF BELFAST, IRELAND, ASSIGNEES  
TO WATSON-WADDELL LIMITED, OF BELFAST, IRELAND, A COMPANY OF NORTHERN  
IRELAND.

## TREATING OR RETTING FIBER-BEARING PLANTS.

No Drawing. Application filed October 31, 1927, Serial No. 230,176, and in Great Britain, September 14, 1927.

The invention relates to the preparing and retting of flax fiber bearing plants to remove therefrom the gum or gumming matter contained in the plant.

5 According to the invention the treating or retting is effected by subjecting the fiber in the form of rove to the action of yeast and/or other fermenting bacteria in a liquid bath with or without dilutions of acids such as 10 sulphurous acid or compounds or extracts of sulphur. The ferment may be carried out at a temperature of 70° to 80° F.

As applied to flax grown for fiber, the fiber prior to retting is spun or twisted into 15 a rove and the rove is immersed in water containing yeast (with or without other substances) and/or aerobic or an aerobic bacteria. The rove may be wound in an open state on to a reel fitted or mounted upon a 20 rove bobbin or other support. Or it may be treated in hank form or wound on a bobbin perforated or otherwise or the rove may be drawn through a trough or vat containing water and yeast on its way to a spinning 25 frame.

As applied to flax grown for seed the plant is after drying with heat threshed and carded in the same machine being deseeded and the woody material removed at the same operation and the fiber therefrom carded or rubbed 30 into a sliver and twisted into a rove and the rove so formed retted in a solution of yeast or other ferments as above described.

In either case the rove may be subsequently

boiled or bleached if desired and after retting 35 it may be treated with a preservative such as a tar product to prevent further fermentation. This rove so retted may be placed in the creel of a spinning frame and drawn through the trough and spun in the usual way or 40 dried and softened and spun on dry spinning frame.

The retting by means of yeast is carried out in a bath of from 70° to 80° F. and will produce alcohol in such quantities as may 45 form a profitable by-product.

What we claim as our invention and desire to protect by Letters Patent is:—

1. Process for retting flax consisting in spinning the fiber into a rove and immersing 50 the rove in water containing yeast.

2. Process for retting flax consisting in spinning the fiber into a rove and immersing the rove in water containing yeast and sulphurous acid. 55

3. Process for retting flax consisting in spinning the fiber into a rove and immersing the rove in water containing yeast, other fermenting bacteria and sulphurous acid.

4. Process for retting flax consisting in 60 spinning the fiber into a rove and immersing the rove in water at a temperature of 70° to 80° F. containing yeast, other fermenting bacteria and sulphurous acid.

In testimony whereof we have hereunto set 65 our hands.

MARTIN WADDELL.  
HENRY COWAN WATSON.